

# United States Patent Office

3,083,088

Patented Mar. 26, 1963

1

3.083.088

**LEADED GASOLINE CONTAINING AROMATIC-  
SUBSTITUTED ESTERS**

Dennis R. Carlson, Park Forest, Everett N. Case, Homewood, and Seymour H. Patinkin, Chicago, Ill., assignors, by mesne assignments, to Sinclair Research Inc., New York, N.Y., a corporation of Delaware

New York, N.Y., a corporation of Delaware  
No Drawing. Filed June 15, 1960, Ser. No. 36,150  
8 Claims. (Cl. 44-69)

9 Claims. (Cl. 44-69)

This invention relates to an improved gasoline composition which is of high octane number, which contains a lead compound as an anti-knocking agent, and also contains an octane rating booster.

By and large, modern gasolines for use in spark-ignited internal combustion engines, e.g., automotive and airplane engines have an octane number of at least 85 RON, that is, as determined by the research method. Almost without exception producers of gasoline use non-hydrocarbon agents to raise the octane number of the gasoline to suppress knocking. Generally this agent is an alkyl lead compound especially a tetra- lower alkyl lead, usually a small amount within the range from about 0.5 to 3.0 cc. per gallon, or even as much as approximately 5 or 6 cc. per gallon. Tetra-ethyl lead is the most widely used anti-knock agent, and is effective in raising the octane and thereby reducing the knock caused by abnormal combustion of gasoline of inferior octane rating. Other lead compounds, such as the lower-alkyl lead carboxylates disclosed in copending application S.N. 855,006, filed November 24, 1959, are useful as anti-knock agents. However, the quantity of lead compound which may be used in a gasoline is limited by decreasing effectiveness at higher percentages, and by the fact that lead compounds cause lead-containing deposits in the cylinders as well as by economic, health and legal considerations.

Several methods are used for determining the octane rating of a gasoline and each method usually gives a different figure; for example, the motor method of determining octane rating generally gives a lower figure than the research method. The spread between the two figures is termed the "sensitivity" of the fuel. Gasolines are sold on the basis of their research octane number but the make of the car and the type of driving determines whether it operates closer to the motor method or research method rating; however, the road octane is usually, numerically, in the space between the two. A gasoline having motor method and research method octane numbers which are closer is less sensitive in its performance to variations in operating conditions.

In accordance with this invention, certain gasoline-compatible, i.e., soluble, miscible or dispersible, aromatic esters are incorporated in a leaded gasoline as an octane booster. The improvement in the gasoline is sometimes greater in the motor method of determining octane rating and sometimes greater when the octane is determined by the research method. The fuel may have less spread between its research method number and its motor method number, and would accordingly be considered as less sensitive.

The ester incorporated in gasoline according to this invention is a primary or secondary mono- or di-aryl substituted lower alkyl ester of a lower carboxylic acid, that is, one which contains the residues of a lower carboxylic acid and a primary or secondary lower aliphatic alcohol having an aryl substituent. The ester may be represented by the formula:

$$\begin{array}{c} \text{H} \\ | \\ \text{R}_1-\text{C}-\text{C}-\text{O}-\text{C}-\text{R}_3 \\ | \\ \text{H} \\ | \\ \text{R}_2 \end{array}$$

2

in which  $R_3$  is a monovalent hydrocarbon radical, preferably of 1-6 carbon atoms and either or both  $R_1$  and  $R_2$  are hydrocarbon-ring aryl radicals of up to 10 carbon atoms in the ring structure, that is, phenyl or naphthyl.

- 5 If one of  $R_1$  or  $R_2$  is non-aryl, it is a hydrogen or monovalent hydrocarbon radical, e.g. an alkyl radical of 1-4 carbon atoms. The hydrocarbon radicals and the carbon atom adjacent  $R_1$  may be substituted, for example with alkyl, alkoxy or hydroxy. The  $R_3$  group may be aryl or

10 lower alkyl, preferably a lower alkyl group having 1-4 carbon atoms. The selected substituents will usually provide an ester of up to about 20 carbon atoms. The acid residue or acyl group



may be derived from, for example, acetic or benzoic acid and generally will contain 2-10 carbon atoms, preferably 2 to 7 carbon atoms. Exemplary preparations of useable

- 20 esters are as follows:

PREPARATION OF  $\alpha$ -PHENYL ETHYL ACETATE



To a solution of 122 grams (1.0 mole)  $\alpha$ -phenyl ethyl alcohol and 95 grams (1.2 mole) pyridine in 200 ml. anhydrous ether was added dropwise 85 ml. (1.2 mole) acetyl chloride. The reaction occurred immediately with evolution of heat and precipitation of pyridine hydrochloride. The heat of reaction maintained the temperature at 40 to 45° C. through most of the addition. The reaction mixture was allowed to cool to room temperature after which an equal volume of water was added to the reaction mixture to dissolve the pyridine hydrochloride and hydrolyze any unreacted acetyl chloride. The ether solution was washed with dilute  $\text{NaHCO}_3$  solution, and then water, and dried over anhydrous  $\text{MgSO}_4$ . The ether was stripped off and the crude product distilled under reduced pressure.

The fraction boiling at 73° C. at 3.0 mm. Hg (220° C. at 760 mm. Hg) was collected for a 92% yield of  $\alpha$ -phenyl ethyl acetate.

## ANALYSIS

$$\left[ \text{DENSITY } \frac{20}{4} = 1.0268 \right]$$

| 55               | Calc. | Det.  |
|------------------|-------|-------|
| Sap. equiv.----- | 342   | 332.3 |
| Percent C-----   | 73.25 | 73.82 |
| Percent H-----   | 7.33  | 7.34  |

## PREPARATION OF 1,2-DIPHENYL ETHYL ACETATE



To a solution of 50 grams (0.25 mole) 1,2-diphenyl-

ethyl alcohol and 24 grams (0.3 mole) pyridine in 100 ml. anhydrous ether was added dropwise 22 ml. (0.3 mole) acetyl chloride. The reaction occurred immediately evolving heat and precipitating pyridine hydrochloride. The heat of reaction held the temperature at 40-45° C. through most of the addition of acetyl chloride. After cooling the reaction mixture to room temperature an equal volume of water was added to dissolve the pyridine hydrochloride and hydrolyze any unreacted acetyl chloride. The ether solution was washed with dilute  $\text{NaHCO}_3$  solution and then water, and dried over anhydrous  $\text{MgSO}_4$ . After stripping off the ether the crude product was distilled under reduced pressure.

The fraction boiling at 122° C. at 0.8 mm. Hg (319° C. at 760 mm. Hg) (reported Hauser, Shivers and Skell, JACS 67, 409-412 [1945], B.P. 312° C. at 760 mm. Hg) was collected for a 75% yield of 1,2-diphenyl ethyl acetate.

## ANALYSIS

$$[\text{DENSITY } \frac{20}{4} = 1.0794]$$

|             | Calc. | Det.  |
|-------------|-------|-------|
| Sap. equiv. | 234   | 210   |
| Percent C.  | 80.00 | 80.46 |
| Percent H.  | 6.67  | 6.78  |

The ester is included in the gasoline composition in the ratio of from about 1 to 50 moles of ester per mole of lead compound and sufficient to increase the octane number of the leaded gasline. The molar ratio of ester to lead compound is preferably about 2 to 40. In terms of volume, the fuel usually contains about 0.1 to 3 volume percent of the ester, preferably about 0.2 to 1.5%, and in amount sufficient to increase the octane rating of the fuel. The concentration of the additive is important in that larger percentages may decrease the octane rating of the gasoline below the rating of the base fuel. Also, the optimum range of effectiveness of the octane booster varies with the lead content of the gasoline. In general, with greater amounts of, for example, tetraethyl lead, not only is the octane increased, but the octane boosting ability of the ester is also increased and the optimum range for this additive is slightly raised.

Gasolines are usually blends of low boiling mineral oil hydrocarbon fractions derived by distillation, cracking, and other refining and chemical conversion processes practiced upon crude petroleum. The gasoline will contain varying proportions of paraffins, olefins, naphthenes and aromatics and generally will boil primarily in the range of about 100 to 425° F. The gasoline of this invention has aromatic components which are at least about 30 volume percent, preferably at least about 40 percent of the hydrocarbon fuel. A typical premium gasoline besides a small amount of lower-alkyl lead compound as an anti-knock agent, may also contain small amounts of other non-hydrocarbon constituents used to impart various properties to the gasoline in its use in internal combustion engines, e.g. scavengers, corrosion inhibitors, etc. Such gasolines frequently have a research method octane number of about 90 to 105 and a motor method octane number of about 80-98. The most widely used tetra-lower-alkyl lead compound added to gasolines as an anti-knock agent is tetra-ethyl lead. "TEL Motor Mix" is used in commercial practice to add tetraethyl lead and scavengers to the gasoline. "Motor Mix" contains 59.2% tetra-ethyl lead, 13.0% ethylene dibromide, 23.9% ethylene dichloride and 3.9% hydrocarbon diluent, dyes, etc. Several gasoline blends were used in the examples and tests reported below. Base gasoline M was a naphtha reformate distillation tower bottoms fraction which had an API gravity of 34.1

and contained 25.1% paraffins, 3.2% naphthenes and 71.7% aromatics. The fraction had an ASTM distillation of:

|      |      |         |      |
|------|------|---------|------|
| 5    | IBP  | ° F.    | 313  |
| 50%  |      | ° F.    | 334  |
| 90%  |      | ° F.    | 368  |
| EP   |      | ° F.    | 442  |
| Rec. |      | percent | 98.5 |
| Res. |      | do      | 1.0  |
| 10   | Loss | do      | 0.5  |

Gasoline blend D comprised 28.4% of these tower bottoms, 28.4% light fluid catalytically cracked gasoline, 19.0% mixed xylenes, 19.0% alkylate fuel and 5.2% butane. This gasoline had an API gravity of 53.0 and a bromine number of 35.0. It analyzed as 34.9% paraffins, 15.1% olefins, 7.1% naphthenes and 42.9% aromatics.

Its ASTM distillation was:

|     |              |      |      |
|-----|--------------|------|------|
| 20  | IBP          | ° F. | 92   |
| 10% |              | ° F. | 133  |
| 50% |              | ° F. | 256  |
| 90% |              | ° F. | 329  |
| EP  |              | ° F. | 403  |
| 25  | Percent rec. |      | 98.0 |
|     | Percent res. |      | 1.0  |
|     | Percent loss |      | 1.0  |

Gasoline blend E had a bromine number of 38.5 and an API gravity of 50.7 and an ASTM distillation of:

|     |      |      |     |
|-----|------|------|-----|
| IBP | ° F. | 103  |     |
| 5%  | ° F. | 103  |     |
| 20% | ° F. | 188  |     |
| 35  | 50%  | ° F. | 272 |
|     | 70%  | ° F. | 306 |
|     | EP   | ° F. | 408 |

It contained the following components ( $\pm 5\%$ ):

|                                            | Percent |
|--------------------------------------------|---------|
| Full-range straight run naphtha reformate  | 30      |
| Light fluid catalytically cracked gasoline | 30      |
| Heavy straight-run naphtha reformate       | 30      |
| Butane                                     | 10      |

and analyzed as

|            | Vol. percent            |        |
|------------|-------------------------|--------|
| Paraffins  | 34.3                    |        |
| Olefins    | 27.2                    |        |
| Naphthenes | 4.7                     |        |
| 50         | Aromatics               | 33.8   |
|            | Sulfur (weight percent) | 0.0213 |

Samples of these base gasolines were obtained and mixed with varying amounts of tetraethyl lead and phenyl-substituted lower alkyl esters of lower carboxylic acids. The octane determinations for each sample are reported in Table I below. Samples 1-6 and 71-76 contained 2.9 cc./gal. TEL added as Motor Mix. Samples 11-16 and 41-46 contained 3 cc./gal. of pure tetraethyl lead. The rest of the samples contained 6 cc./gal. of pure tetraethyl lead.

Table I  
BASE: BLEND E (2.9 CC. TEL/GAL.)

| 65 | Sample | Additive                       | Vol. percent | Octane       |                 | Change from base |                 |
|----|--------|--------------------------------|--------------|--------------|-----------------|------------------|-----------------|
|    |        |                                |              | Motor method | Research method | Motor method     | Research method |
| 70 | 1      | None                           |              | 88.5         | 99.5            | -0.1             | +0.1            |
|    | 2      | $\alpha$ -phenyl ethyl acetate | 0.25         | 88.4         | 99.6            | -0.1             | +0.1            |
|    | 3      | do                             | 0.50         | 88.4         | 99.7            | -0.1             | +0.2            |
|    | 4      | do                             | 0.75         | 88.5         | 99.8            | 0                | +0.3            |
|    | 5      | do                             | 1.00         | 88.4         | 99.9            | -0.1             | +0.4            |
|    | 6      | do                             | 1.25         | 88.5         | 99.7            | 0                | +0.2            |

Table I—Continued

BASE: BLEND D (3 CC. TEL/GAL.)

| Sample | Additive                       | Vol. percent | Octane       |                 | Change from base |                 |
|--------|--------------------------------|--------------|--------------|-----------------|------------------|-----------------|
|        |                                |              | Motor method | Research method | Motor method     | Research method |
| 11     | None                           |              | 92.4         | 103.5           |                  |                 |
| 12     | $\alpha$ -phenyl ethyl acetate | 0.25         | 92.7         | 103.7           | +0.3             | +0.2            |
| 13     | do                             | 0.50         | 92.7         | 103.5           | +0.3             | 0               |
| 14     | do                             | 0.75         | 92.6         | 103.9           | +0.2             | +0.4            |
| 15     | do                             | 1.00         | 92.5         | 104.0           | +0.1             | +0.5            |
| 16     | do                             | 1.25         | 92.7         | 104.2           | +0.3             | +0.7            |

BASE: BLEND D (6 CC. TEL/GAL.)

|    |                                |      | 95.0 | 106.1 |      |      |
|----|--------------------------------|------|------|-------|------|------|
|    |                                |      | 96.0 | 106.3 | +1.0 | +0.2 |
| 21 | None                           |      |      |       |      |      |
| 22 | $\alpha$ -phenyl ethyl acetate | 0.50 |      |       |      |      |
| 23 | do                             | 0.75 | 97.3 | 106.7 | +2.3 | +0.6 |
| 24 | do                             | 1.00 | 96.4 | 106.6 | +1.4 | +0.5 |
| 25 | do                             | 1.25 | 97.3 | 106.8 | +2.3 | +0.7 |
| 26 | do                             | 1.50 | 96.7 | 106.8 | +1.7 | +0.7 |

BASE: BLEND D (6 CC. TEL/GAL.)

|    |                                |      | 94.5 | 105.9 |      |      |
|----|--------------------------------|------|------|-------|------|------|
|    |                                |      | 96.6 | 107.4 | +2.1 | +1.5 |
| 31 | None                           |      |      |       |      |      |
| 32 | $\alpha$ -phenyl ethyl acetate | 1.75 |      |       |      |      |
| 33 | do                             | 2.00 | 96.9 | 107.4 | +2.4 | +1.5 |
| 34 | do                             | 2.25 | 96.7 | 107.3 | +2.2 | +1.4 |
| 35 | do                             | 2.50 | 97.1 | 107.1 | +2.6 | +1.2 |
| 36 | do                             | 2.75 | 96.6 | 107.1 | +2.1 | +1.2 |
| 37 | do                             | 3.00 | 96.3 | 107.0 | +1.8 | +1.1 |

BASE: FRACTION M (3 CC. TEL/GAL.)

|    |                                |      | 92.1 | 102.4 |      |      |
|----|--------------------------------|------|------|-------|------|------|
|    |                                |      | 92.3 | 102.5 | +0.2 | +0.1 |
| 41 | None                           |      |      |       |      |      |
| 42 | $\alpha$ -phenyl ethyl acetate | 0.50 |      |       |      |      |
| 43 | do                             | 0.75 | 92.8 | 102.7 | +0.7 | +0.3 |
| 44 | do                             | 1.00 | 93.0 | 102.7 | +0.9 | +0.3 |
| 45 | do                             | 1.25 | 92.8 | 102.8 | +0.7 | +0.4 |
| 46 | do                             | 1.50 | 92.8 | 102.7 | +0.7 | +0.3 |

BASE: FRACTION M (6 CC. TEL/GAL.)

|    |                               |      | 94.3 | 103.4 |      |      |
|----|-------------------------------|------|------|-------|------|------|
|    |                               |      | 94.9 | 103.7 | +0.6 | +0.3 |
| 51 | None                          |      |      |       |      |      |
| 52 | $\beta$ -phenyl ethyl acetate | 1.25 |      |       |      |      |
| 53 | do                            | 1.50 | 95.1 | 103.6 | +0.8 | +0.2 |
| 54 | do                            | 1.75 | 94.8 | 103.6 | +0.5 | +0.2 |
| 55 | do                            | 2.00 | 95.1 | 103.5 | +0.8 | +0.1 |
| 56 | do                            | 2.25 | 95.6 | 103.8 | +1.3 | +0.4 |
| 57 | do                            | 2.50 | 95.7 | 103.8 | +1.4 | +0.4 |
| 58 | do                            | 2.75 | 95.0 | 103.7 | +0.7 | +0.3 |
| 59 | do                            | 3.00 | 95.5 | 103.6 | +1.2 | +0.2 |

BASE: BLEND D (6 CC. TEL/GAL.)

|    |                               |      | 95.1 | 105.7 |      |      |
|----|-------------------------------|------|------|-------|------|------|
|    |                               |      | 94.9 | 105.5 | -0.2 | -0.2 |
| 61 | None                          |      |      |       |      |      |
| 62 | $\beta$ -phenyl ethyl acetate | 0.50 |      |       |      |      |
| 63 | do                            | 0.75 | 95.3 | 105.7 | +0.2 | 0    |
| 64 | do                            | 1.00 | 95.4 | 105.7 | +0.3 | 0    |
| 65 | do                            | 1.25 | 95.8 | 105.9 | +0.7 | +0.2 |
| 66 | do                            | 1.50 | 96.0 | 105.9 | +0.9 | +0.2 |
| 67 | do                            | 1.75 | 95.6 | 105.7 | +0.5 | 0    |
| 68 | do                            | 2.00 | 95.9 | 106.0 | +0.8 | +0.3 |

BASE: BLEND E (2.9 CC. TEL/GAL.)

|    |                            |      | 88.4 | 99.4 |      |      |
|----|----------------------------|------|------|------|------|------|
|    |                            |      | 88.6 | 99.5 | +0.2 | +0.1 |
| 71 | None                       |      |      |      |      |      |
| 72 | 1,2-diphenyl ethyl acetate | 0.50 |      |      |      |      |
| 73 | do                         | 0.75 | 88.6 | 99.4 | +0.2 | 0    |
| 74 | do                         | 1.00 | 88.5 | 99.5 | +0.1 | +0.1 |
| 75 | do                         | 1.25 | 88.8 | 99.6 | +0.4 | +0.2 |
| 76 | do                         | 1.50 | 88.8 | 99.6 | +0.4 | +0.2 |

BASE: BLEND D (6 CC. TEL/GAL.)

|    |                            |      | 94.9 | 105.6 |      |      |
|----|----------------------------|------|------|-------|------|------|
|    |                            |      | 95.8 | 106.0 | +0.9 | +0.4 |
| 81 | None                       |      |      |       |      |      |
| 82 | 1,2-diphenyl ethyl acetate | 1.50 |      |       |      |      |
| 83 | do                         | 1.75 | 96.3 | 106.3 | +1.4 | +0.7 |
| 84 | do                         | 2.00 | 97.1 | 106.2 | +2.2 | +0.6 |
| 85 | do                         | 2.25 | 98.0 | 106.3 | +3.1 | +0.7 |

Table I—Continued

BASE: BLEND D (6 CC. TEL/GAL.)

| 5  | Sample | Additive                         | Vol. percent | Octane       |                 | Change from base |                 |
|----|--------|----------------------------------|--------------|--------------|-----------------|------------------|-----------------|
|    |        |                                  |              | Motor method | Research method | Motor method     | Research method |
| 91 | 91     | None                             | 1.0          | 94.3         | 106.5           |                  |                 |
| 92 | 92     | $\beta$ -phenyl ethyl propionate | 1.25         | 95.4         | 106.7           | +1.1             | +0.2            |
| 93 | 93     | do                               | 1.5          | 94.8         | 106.9           | +0.5             | +0.4            |
| 94 | 94     | do                               | 1.75         | 94.9         | 107.1           | +0.6             | +0.6            |
| 95 | 95     | do                               | 2.0          | 95.5         | 107.3           | +1.2             | +0.8            |
| 96 | 96     | do                               | 2.0          | 95.2         | 107.3           | +0.9             | +0.8            |

BASE: BLEND D (6 CC. TEL/GAL.)

| 15  | Sample | Additive                       | Vol. percent | Octane       |                 | Change from base |                 |
|-----|--------|--------------------------------|--------------|--------------|-----------------|------------------|-----------------|
|     |        |                                |              | Motor method | Research method | Motor method     | Research method |
| 101 | 101    | None                           | 1.0          | 94.5         | 106.4           |                  |                 |
| 102 | 102    | $\beta$ -phenyl ethyl butyrate | 1.0          | 95.1         | 106.6           | +0.6             | +0.2            |
| 103 | 103    | do                             | 1.25         | 95.1         | 106.9           | +0.6             | +0.5            |
| 104 | 104    | do                             | 1.5          | 95.0         | 106.7           | +0.5             | +0.3            |
| 105 | 105    | do                             | 1.75         | 95.1         | 106.7           | +0.6             | +0.3            |
| 106 | 106    | do                             | 2.0          | 95.0         | 106.9           | +0.5             | +0.5            |

BASE: FRACTION M (6 CC. TEL/GAL.)

| 25  | Sample | Additive                       | Vol. percent | Octane       |                 | Change from base |                 |
|-----|--------|--------------------------------|--------------|--------------|-----------------|------------------|-----------------|
|     |        |                                |              | Motor method | Research method | Motor method     | Research method |
| 111 | 111    | None                           | 1.25         | 94.2         | 103.0           |                  |                 |
| 112 | 112    | $\beta$ -phenyl ethyl benzoate | 1.25         | 94.7         | 103.4           | +0.5             | +0.4            |
| 113 | 113    | do                             | 1.50         | 94.7         | 103.4           | +0.5             | +0.4            |
| 114 | 114    | do                             | 1.75         | 94.7         | 103.5           | +0.5             | +0.6            |
| 115 | 115    | do                             | 2.00         | 95.2         | 103.6           | +1.0             | +0.6            |
| 116 | 116    | do                             | 2.25         | 95.6         | 103.7           | +1.4             | +0.7            |
| 117 | 117    | do                             | 2.50         | 95.4         | 103.6           | +1.2             | +0.6            |
| 118 | 118    | do                             | 2.75         | 95.4         | 103.5           | +1.2             | +0.5            |

30 The above examples, which are to be considered illustrative only and not limiting, show that the addition of the enumerated esters to a leaded gasoline boosts the octane rating of gasoline fuels.

It is claimed:

35 1. A leaded gasoline consisting essentially of base hydrocarbon gasoline containing at least about 30% aromatic hydrocarbons, a small amount of lower alkyl lead anti-knock agent sufficient to reduce knock and about 1 to 50 moles per mole of lead compound and sufficient to improve the octane rating of the leaded gasoline of a gasoline-compatible aryl substituted lower alkyl ester of a lower carboxylic acid of up to about 20 carbon atoms and having the formula:

50 in which  $\text{R}_3$  is a monovalent hydrocarbon radical,  $\text{R}_1$  and  $\text{R}_2$  are selected from the group consisting of hydrogen and monovalent hydrocarbon radicals, with the proviso that at least one of  $\text{R}_1$  and  $\text{R}_2$  is a hydrocarbon-ring aryl radical of up to 10 carbon atoms in the ring structure.55 2. A gasoline composition according to claim 1 in which  $\text{R}_3$  has 1 to 6 carbon atoms.

56 3. A gasoline composition according to claim 1 containing about 2 to 40 moles of ester per mole of lead compound.

57 4. A gasoline composition according to claim 1 containing at least about 40% aromatic hydrocarbons.

58 5. A gasoline composition according to claim 3, containing at least about 40% aromatic hydrocarbons in which the ester is an acetate.

59 6. A gasoline composition according to claim 5 in which the ester is  $\alpha$ -phenyl ethyl acetate.60 7. A gasoline composition according to claim 5 in which the ester is  $\beta$ -phenyl ethyl acetate.

61 8. A gasoline composition according to claim 5 in which the ester is 1,2-diphenyl ethyl acetate.

62 9. A gasoline composition according to claim 5 in which the ester is  $\beta$ -phenyl ethyl benzoate.

63 10. A gasoline composition according to claim 5 in which the ester is 1,2-diphenyl ethyl acetate.

## References Cited in the file of this patent

## FOREIGN PATENTS

42,139 Australia ----- Oct. 8, 1958  
571,921 Belgium ----- Oct. 10, 1958